

## UNITED STATES PATENT OFFICE

2,375,485

## LUBRICATING GREASES

John D. Morgan, South Orange, and Russell E. Lowe, East Orange, N. J., assignors to Cities Service Oil Company, New York, N. Y., a corporation of Pennsylvania

No Drawing. Application August 10, 1943,  
Serial No. 498,082

4 Claims. (Cl. 252—36)

This invention relates to greases. More particularly the invention relates to greases having a substantially uniform viscosity at the usual working temperatures.

For the operation of gun turrets it is important that the lubricant, which is a grease, shall have a substantially uniform viscosity throughout the temperature range of the parts on which it is used. The rollers and pinions of a gun turret usually operate in the temperature range of 35° to 80° F. It is important also that the grease shall adhere to the parts and shall have a uniform consistency in the temperature range of use.

The primary object of the present invention is to provide a grease which will cling to the parts to be lubricated and will have a comparatively uniform viscosity in the temperature range of 35° to 80° F.

Another object of the invention is to provide a grease which will be non-corrosive to steel pinions and rollers as well as copper parts.

The United States Navy places a very rigid specification on greases which are to be used on gun turrets because these turrets must operate properly under very severe operating conditions. The specification requires a uniform consistency with a dropping point of 250° F. minimum, a work penetration of 330 to 350 at 77° F. and a work penetration of 280 minimum at 40° F. This lubricant shall be only slightly corrosive to copper and non-corrosive on steel. Furthermore the grease must cling to the steel parts on which it is applied.

A grease which will meet these specifications has been found to have the following composition:

|                        | Percent by weight |
|------------------------|-------------------|
| Calcium stearate       | 7                 |
| Lithium stearate       | 2                 |
| Aluminum tri-stearate  | 0.6               |
| Lead oleate            | 1                 |
| Mid-Continent pale oil | 67                |
| Naphthenic oil         | 22.4              |

The proportions in which the above-mentioned ingredients are mixed and the method of making the grease is critical, particularly if the Navy specifications are to be met. In order to successfully make this grease the Mid-Continent neutral oil is mixed with the naphthenic oil and then the stearates are dissolved in the oil while the entire mass is thoroughly agitated at room temperatures. After the stearates are thoroughly mixed and blended with the oils, the lead oleate

is added to the mixture and thoroughly blended therewith. Thereafter the mixture is constantly agitated while being heated to a maximum of 420° F. Foaming of the mixture starts at 250° F. and the foam breaks at about 390° F. The volume of foam is about equal to the volume of liquid. The mixture of foam and liquid is then rapidly chilled to form the grease. The chilling is preferably accomplished by passing it over a chilling roll or placing it in layers in shallow pans, the layer being approximately one-sixteenth of an inch thick.

The Mid-Continent neutral oil is preferably an oil of #3 color and having a viscosity of 400 at 100° F. The naphthenic oil is a pale oil having a viscosity of 1200 at 100° F.

The calcium stearate and lead oleate have the effect of making the grease soft. The aluminum stearate is very effective in making a uniform blend of the soaps in the oils and prevents the mixture from breaking. The lead oleate acts effectively also as a corrosion inhibitor to prevent the grease from corroding either copper or steel parts.

25 A grease manufactured in accordance with the above process when the ingredients are used in the proportions mentioned above, has substantially the following specification:

|                            |             |
|----------------------------|-------------|
| Consistency                | Homogeneous |
| Dropping point             | ° F. 254    |
| Work penetration at 77° F. | 338         |
| Work penetration at 40° F. | 320         |
| Adhesion to steel          | Complete    |
| Corrosion to copper        | None        |
| Corrosion to steel         | None        |

The specification which has been set by the Navy is quite rigid in order to have the grease maintain a substantially uniform viscosity throughout the working range and also provide a grease which will cling to the steel and not drop from the parts being lubricated while the turret is in operation.

The preferred form of the invention having been thus described what is claimed as new is:

1. A turret lubricating grease, comprising about 7% by weight of calcium stearate, about 2% by weight of lithium stearate, about 0.6% by weight of aluminum stearate, about 1% by weight of lead oleate, the remainder of the lubricant consisting essentially of a mixture of neutral mineral oil and naphthenic oil, said grease being prepared by mixing the stearates with the oils then adding the lead oleate, heating the mixture to a maximum temperature of about 420° F., and then rapidly chilling the mixture.

2. A turret lubricating grease, comprising about 7% by weight of calcium stearate, about 2% by weight of lithium stearate, about 0.6% by weight of aluminum tristearate, about 1% by weight of lead oleate, the remainder of the lubricant consisting essentially of a mixture of neutral mineral oil and a pale oil in the ratio of about 3 to 1, said grease being prepared by mixing the stearates with the oils then adding the lead oleate, heating the mixture to a maximum temperature of about 420° F., and then rapidly chilling the mixture to produce the grease.

3. A turret lubricating grease, comprising about 67% by weight of a neutral mineral oil having a viscosity of about 400 at 100° F., about 22.4% by weight of a pale mineral oil having a viscosity of about 1200 at 100° F., about 7% by weight of calcium stearate, about 2% by weight of lithium

stearate, about 0.6% by weight of aluminum stearate, and about 1% by weight of lead oleate.

4. The method of manufacturing a turret lubricating grease, which comprises mixing about 67% by weight of a neutral mineral oil with about 22.4% by weight of a pale naphthenic oil, intimately mixing with this oil mixture about 7% by weight of calcium stearate, about 2% by weight of lithium stearate, and about 0.6% by weight of aluminum stearate, thereafter incorporating in the resulting mixture about 1% by weight of lead oleate, heating the final mixture to a maximum temperature of about 420° F., and rapidly chilling the heated mixture to produce the desired grease.

JOHN D. MORGAN.  
RUSSELL E. LOWE.